

Jan. 3, 1939.

L. A. HALL ET AL

2,142,870

ALKALINE DETERGENT COMPOUND

Filed April 30, 1937.

FIG.1.



FIG.2.



Inventors:  
Lloyd A. Hall,  
Carroll L. Griffith,  
By: Benjamin A. Schneider  
Attorneys

## UNITED STATES PATENT OFFICE

2,142,870

## ALKALINE DETERGENT COMPOUND

Lloyd A. Hall and Carroll L. Griffith, Chicago,  
Ill., assignors to The Griffith Laboratories, Inc.,  
a corporation of Illinois

Application April 30, 1937, Serial No. 139,860

14 Claims.

(Cl. 87—5)

The present invention relates to improvements in alkaline compounds and more particularly to partially hydrated alkaline phosphate car-

5 bonate compounds of a new type having a high degree of stability, especially in respect of their water content. The compounds prepared in accordance with the present invention are thus particularly suitable for use as detergents and in the preparation of alkaline detergent mixtures.

10 The alkaline phosphates and especially trisodium phosphate have been found to be highly desirable as detergents and as constituents of detergent compositions, particularly for the removal of oil and grease from iron, steel, tinned and other metal surfaces, and from enamelware, china, glass, stone, concrete and the like. In general, it has been found desirable to combine the trisodium phosphate with other alkalis, such as sodium hydroxide, or with various auxiliary 15 agents, particularly oxidizing agents such as hypochlorites, perborates or the like. The trisodium phosphates, in their usual hydrated forms are, however, unstable in respect of their water content, the dodecahydrate readily giving up water, particularly in dry atmosphere; and the monohydrate tending to take up and collect moisture, particularly in humid atmospheres. Thus, normal changes in humidity of the air in rooms containing opened packages of these materials lead 20 to changes in composition and resulting changes of behavior, to caking or to wetting or deliquescence of the particles, either at and near the surface or throughout the entire mass of the package in some cases or to a greater or less degree of efflorescence in others. In any case, the material becomes unsightly and in many cases unusable.

25 The lack of stability of the moisture content of the trisodium phosphates is also disadvantageous in connection with their use in detergent compositions or admixtures, since it frequently leads to premature reaction and decomposition of the mixture, loss of effectiveness and to unsightliness and unusability of the products.

30 It is an object of the present invention to prepare a trisodium phosphate compound of marked stability, not subject to changes appreciably affecting its physical or chemical characteristics as a result of the temperature and humidity changes to which it may ordinarily be subjected, and capable of forming highly stable detergent compositions or mixtures.

35 In carrying out the present invention, it has been the further objects thereof to maintain the detergent characteristics of trisodium phosphate,

without securing excessive or increased alkalinity or causticity, and to provide a compound of ready and rapid solubility.

In carrying out the present invention, we employ trisodium phosphate together with a sodium carbonate compound of lower hydrogen content than sodium bicarbonate, such as sodium carbonate or sodium sesquicarbonate. It will be noted that the constituents used in carrying out the invention tend to combine with water in substantial proportions to form crystalline compounds.

The alkaline compounds formed in accordance with the present invention are new, stable hydrated compounds of trisodium phosphate and sodium carbonate or sesquicarbonate wherein the water or a portion thereof appears to play a definite role in forming a compound having a distinctive crystalline lattice structure, as shown by the formation of a characteristic X-ray diffraction pattern. The proportion of water present is in general from about 18 to about 25 or 26 percent, although products having the desired characteristics have been formed containing somewhat less amounts of water. Where the characteristic sodium phosphate-carbonate compound of the present invention appears, the water content of the compound, within the range of proportions mentioned, is firmly held and the product shows a high degree of stability, with freedom from caking, deliquescence and efflorescence and forms stable mixtures with other substances readily affected or decomposed by water.

35 In the preparation of the alkaline products of the present invention, the sodium phosphate and sodium carbonate compounds are employed in such molecular proportions as to provide from about 0.5 up to about 1.8 phosphate radicals to each carbonate radical, the preferred ratio being 40 from 1 to 1.25 ( $PO_4$ ) to 1( $CO_3$ ). The sodium phosphate employed may be anhydrous or hydrated trisodium phosphate; the commonly available monohydrate or dodecahydrate may be used. Similarly, the sodium carbonate compound used 45 may be anhydrous soda ash or hydrated sodium carbonate or sesquicarbonate. The selected sodium carbonate and sodium phosphate compounds, in the desired proportions, are mixed with a suitable proportion of water to form a slurry and to 50 wholly or partly dissolve the solid components when heated. I prefer to employ a proportion of water ranging from 45 or 50% to 100% of the weight of the solid components, although more 55 may be used if desired, for example, up to about

150%. Such excess over 45 or 50% of water as may be employed is largely a matter of convenience in operation, and in general the presence of water in excess of 100% of the weight of the solid constituents is to be avoided because of the increased time and expense of evaporation and because in some cases it appears to prevent the formation of the desired hydrated phosphate carbonate complex or compound. As the ratios of phosphate to carbonate approach the upper and lower limits of the ranges set forth, it appears important that lower proportions of water be used in preparing the slurry, substantially below 100% and preferably below 75% of the solids initially used.

The aqueous mixture is then subjected to evaporation over an open flame or on a drum dryer to reduce its water content to a point such that on cooling it rapidly congeals or solidifies. The resulting mass is then broken up, ground or pulverized and dried, suitably at a temperature of 130 to 140° C. and preferably in vacuo, to constant weight.

The products prepared in accordance with the present invention are distinctive in that they contain and consist largely of a hydrated complex sodium phosphate and carbonate compound, and are hence highly stable in respect of their water content. The precise composition of these products may vary to some extent, as some excess of either the carbonate or phosphate compound may be present without appreciably affecting the stability of the product or its rapidity and completeness of solution or effectiveness of utilization.

In respect of the formation of the hydrated complex in accordance with the present invention, it will be noted that both the sodium phosphate and sodium carbonate constituents of the mixture tend to form crystalline hydrates containing considerable proportions of water, and each appears to display a strong avidity for the relatively inadequate proportion of water available. As a result, the resulting product, prepared as herein described, is very stable as to its water content and physical properties, and in each case a definite hydrated compound or complex of sodium phosphate and sodium carbonate is formed.

The products formed in accordance with the present invention are therefore particularly suited for use as commercial detergents, since they remain stable under varying conditions of temperature and humidity, and consequently maintain a constant and uniform physical condition in opened and partly used packages. They may be prepared as stable powders of any desired degree of fineness which are rapidly soluble and do not cake or become wet in opened packages. They are also excellent water softeners and improve the lathering qualities of soaps and the permanence of the lathers formed. As they are non-caustic, they do not injuriously affect the hands and skin of users.

The products of the present invention have but slight corrosive action upon tin and other metals (other than aluminum) commonly used as containers for culinary purposes, in dairies, bakeries and the like. They are rapid and effective in their detergent action and in the removal of oily and greasy deposits, and are thus particularly useful in the cleaning of cooking, baking and dairy pans, vessels and utensils and in the cleaning of metal work, stone and cement and the like.

By reason of their stability, the products of the

present invention are also adapted to form detergent mixtures or compositions in admixture with other substances, particularly those which are readily affected or decomposed by moisture and hence cannot ordinarily be used with phosphates, carbonates and other detergent alkalies which readily yield a part of their moisture content or which tend to deliquesce in humid atmosphere.

This hydrated complex or compound of sodium phosphate and sodium carbonate prepared in accordance with the present invention has a distinctive and identifiable structure, as is clearly indicated by its X-ray diffraction pattern. The compounds prepared in accordance with the present invention, when subjected to crystal analysis by X-ray diffraction, preferably by the powder method, display an unique crystal lattice spacing which is different and distinguishable from those of compounds hitherto known. Since, as is now well established, each crystalline substance is distinguishable by the kind and arrangement of the atoms and molecules making up the crystal and by the spacing between them; and that on passing an X-ray beam through the substance and permitting the diffracted beams to act on a photographic film or plate, a pattern is secured which is characteristic of the substance. By passing a monochromatic beam of X-rays through a compacted powder mass and recording the diffracted rays upon a flat photographic emulsion surface having its plane perpendicular to the incident beam, the diffracted beams will be recorded as a series of rings of varying spacings and intensities surrounding the central spot formed by the incident beam. By using a photographic emulsion surface or film in the form of a cylindrical section with its axis perpendicular to the incident beam, on opening or unrolling the film, the diffracted beams will be recorded as lines spaced from the position of the incident beam. The resulting patterns or traces in either case are characteristic and the definite lines and spacings of lines corresponding to definite crystalline substance, including hydrated complexes, as pointed out, for example, in "Applied X-rays" by George L. Clark (2nd ed., 1932, New York), pages 226 to 228 and 252, 253.

In the accompanying drawing are illustrated diagrammatically the principal lines and spacing of the lines of X-ray diffraction patterns secured from powdered compounds prepared in accordance with the present invention, as hereinafter described. In the drawing:

Figure 1 shows diagrammatically the pattern obtained on use of a cylindrical cassette, the principal lines being indicated by straight lines; and

Fig. 2 shows diagrammatically the corresponding lines of the pattern as recorded on a flat film.

The characteristic lines and spacings of the patterns illustrated in the drawing are secured from products formed in accordance with my invention and will be fully described hereinafter in connection with certain specific examples of the production thereof.

Example No. 1.—750 pounds of trisodium phosphate (crystalline) and 180 pounds of sodium sesquicarbonate are dissolved in about 100 gallons of water by heating to about 200° F. to effect solution. The mixture is then subjected to rapid drying. Although in smaller quantities the drying or evaporation may readily be effected in open fired pans, in larger quantities it is preferred that the heating and drying be effected, for example, on a drying drum, suitably at a temperature above 300° F. After the drying operation.

the mass, which is in a fused or molten condition, is allowed to cool, and sets or congeals into a hard mass. This mass is then broken up and dried at a temperature of 105 to 110° C. to constant weight. The resulting product is then powdered. It is found to contain about 20% of water in combined form or as water of hydration. It is a stable compound, does not change or alter its characteristics nor cake on standing with changes in temperature and is rapidly soluble and has excellent detergent qualities. On X-ray analysis it records diffraction patterns having the principal characteristic lines and spacings as illustrated diagrammatically on the figures of the accompanying drawing, in which Fig. 1 shows the characteristic pattern as recorded on a cylindrical film and Fig. 2 as recorded on a flat film.

The diagrammatic illustrations in the drawing show only the principal characteristic lines and their spacings and these lines may best be identified by reference to the corresponding crystal lattice spacings in Angstrom units according to the Bragg formula:

$$n\lambda=2d \sin \theta$$

in which  $n$  is an integer, and represents the order of the diffraction;  $\lambda$  is the wave length of the radiation used;  $d$  is the crystal lattice spacing and  $2\theta$  is the angle of diffraction. In the instant case, the radiation used is the  $K_{\alpha}$  beam from a copper anticathode having a wave length of 1.539 A. U.

Referring to the drawing, the lines corresponding to the same lattice spacings  $d$  in the two figures are indicated by the same numerals, as follows:

| Line No. | Spacings corresponding to line centers (in A. U.) |
|----------|---------------------------------------------------|
| 1        | 5.863                                             |
| 2        | 5.423                                             |
| 3        | 4.727±0.005                                       |
| 4        | 4.379±0.004                                       |
| 5        | 4.218                                             |
| 6        | 3.882±0.01                                        |
| 7        | 3.312±0.005                                       |
| 8        | 3.067±0.001                                       |

The principal figures given for the spacings listed may be regarded as accurate to 0.01 A. U. ( $10^{10}$  cm.).

In the patterns illustrated, the lines designated 9 to 12 inclusive are characteristic of hydrated sodium carbonate and indicate the presence thereof to a minor undetermined proportion in the product prepared as described in Example No. 1.

It will be understood that the width of the characteristic lines will vary with the size of 60 grain of the powder subjected to analysis, and their uniformity with the extent to which the sample is compacted, the uniformity of grain size and the like.

In the preparation of the product as hereinbefore described the molecular ratio of the phosphate to the sesquicarbonate is approximately 3.6 to 1; and since the sesquicarbonate contains three carbonate radicals, the ratio of phosphate radicals to carbonate radicals is approximately 70 1.2 to 1.

*Example No. 2.*—Normal trisodium phosphate, sodium carbonate and water are admixed in the proportions of 2 parts by weight of the phosphate, 1 of the anhydrous carbonate and 3 of water, giving an initial ratio of 0.56 phosphate group

to 1 carbonate group. Instead of the normal trisodium phosphate, an equivalent amount (about 0.96 part) of the monohydrated compound may be used. Solution is effected by heating the mixture, which is then dehydrated on a drying drum as in the case of Example No. 1 or by heating in a shallow evaporating pan until sputtering ensues, after which drying is continued at a temperature of 105–110° C. The final product is suitably ground or powdered for use, and is essentially similar in its properties and stability to the product made in accordance with Example No. 1. It contains 25.74% water (determined at 140° C.) and on X-ray analysis yields a diffraction pattern having the same characteristic lines and spacings as those of the product of Example No. 1.

*Example No. 3.*—3 parts by weight of the monohydrated trisodium phosphate, 1 of sodium sesquicarbonate and 2 of water are mixed, heated to effect partial solution of the resulting slurry, and dried or dehydrated as described in connection with Example No. 2. The initial ratio of phosphate radicals to carbonate radicals is 1.8 to 1. The resulting product has a moisture content of about 23.2%.

The product of Example 3 is likewise stable and shows on X-ray analysis the characteristic diffraction pattern illustrated in the drawing in connection with the product of Example No. 1. By reason of the high phosphate ratio of this product, the lines characteristic of the phosphates may accompany it.

In preparing the alkaline products of the present invention, anhydrous or monohydrated trisodium phosphate may be employed as well as the normal crystalline compound, and anhydrous or crystalline sodium carbonate or sesquicarbonate may be employed. The proportions of these constituents employed may be varied and in some cases the proportion of phosphate compound has been increased to provide a ratio of phosphate groups to carbonate groups of almost 2:1 while maintaining to a large extent the stability of the product. In general, while such products, on X-ray analysis, show the characteristic diffraction pattern of the product of the present invention as hereinbefore described, they may also show that characteristic of unreacted sodium phosphates.

Although the present invention has been described in connection with the details of specific examples embodying the same, it is not intended that these details shall be regarded as limitations on the scope of the invention, except in so far as included in the accompanying claims.

We claim:

1. The method of forming a stable alkaline detergent compound comprising principally a hydrated sodium phosphate and carbonate complex which comprises admixing a trisodium phosphate and a sodium carbonate compound of the class consisting of sodium carbonate and sodium sesquicarbonate and their hydrates in proportions to provide a ratio of about 0.5 to about 1.8 phosphate groups to each carbonate group with water in proportions of from about 45% upwardly of said solid compounds to at least form a slurry and dehydrating the resulting mixture to form a stable, normally solid, pulverizable product, containing in stable combination from about 18 to about 26% of water.

2. The method of forming a stable alkaline detergent compound comprising principally a hydrated sodium phosphate and carbonate com-

plex which comprises admixing a trisodium phosphate and a sodium carbonate compound of the class consisting of sodium carbonate and sodium sesquicarbonate and their hydrates in proportion 5 to provide a ratio of 0.5 to 1.8 phosphate groups to each carbonate group, dissolving the mixture in water and dehydrating the resulting mixture to form a normally solid pulverizable product containing in stable combination from about 18 to 10 about 26% of water.

3. The method of forming a stable alkaline detergent compound comprising principally a hydrated sodium phosphate and carbonate complex which comprises admixing a trisodium phosphate 15 and a sodium carbonate compound of the class consisting of sodium carbonate and sodium sesquicarbonate and their hydrates in proportion to provide a ratio of 0.5 to 1.8 phosphate groups to each carbonate group, adding water to the mixture in proportions of from about 45 to about 20 150% by weight of the mixture to at least form a slurry and dehydrating the resulting mixture to form a stable, normally solid pulverizable product containing in stable combination from about 18 to 25 about 26% of water.

4. The method of forming a stable alkaline detergent compound comprising principally a hydrated sodium phosphate and carbonate complex which comprises admixing a trisodium phosphate 30 and a sodium carbonate compound of the class consisting of sodium carbonate and sodium sesquicarbonate and their hydrates in proportion to provide a ratio of 1 to 1.25 phosphate groups to 1 carbonate group, adding water to the mixture 35 in proportions of from about 45 to about 100% by weight of the mixture to at least form a slurry and dehydrating the resulting mixture to form a normally solid, pulverizable product containing in stable combination from about 18 to about 26% 40 of water.

5. The method of forming a stable alkaline detergent compound comprising principally a hydrated sodium phosphate and carbonate complex which comprises dehydrating an aqueous solution 45 containing trisodium phosphate and a sodium carbonate of the class consisting of sodium carbonate and sodium sesquicarbonate in proportion to provide a ratio of 0.5 to 1.8 phosphate groups to each carbonate whereby a stable product principally consisting of a hydrated complex 50 of sodium phosphate and sodium carbonate and containing from about 18 to about 25% of water is secured.

6. The method of forming a stable alkaline detergent compound comprising principally a hydrated sodium phosphate and carbonate complex which comprises dehydrating an aqueous solution 55 containing trisodium phosphate and a sodium carbonate of the class consisting of sodium carbonate and sodium sesquicarbonate in proportion to provide a ratio of 1 to 1.25 phosphate groups to each carbonate group whereby a stable product principally consisting of a hydrated complex 60 of sodium phosphate and sodium carbonate and containing from about 18 to about 25% of water is secured.

7. The method of forming a stable alkaline detergent compound comprising principally a hydrated sodium phosphate and carbonate complex which comprises heating 750 parts of normal trisodium phosphate and 180 parts of sodium sesquicarbonate with water to effect solution thereof, and dehydrating the mixture, there-

by forming a stable product containing about 20% of water and consisting principally of a hydrated compound of sodium phosphate and sodium carbonate.

8. The method of forming a stable alkaline detergent compound comprising principally a hydrated sodium phosphate and carbonate complex which comprises heating an aqueous solution containing trisodium phosphate and anhydrous sodium carbonate in proportions equivalent to 2 10 parts of normal trisodium phosphate to 1 of sodium carbonate to dehydrate the same to form a stable product containing about 25.74% of water and consisting largely of a hydrated compound of sodium phosphate and sodium car- 15 bonate.

9. As a new product, a readily soluble, non-caking non-hygroscopic alkaline detergent material consisting principally of a hydrated complex of trisodium phosphate and sodium carbonate, said product containing from about 18 to about 26% of water in stable combination and having initially a ratio of from 0.5 to 1.8 phosphate groups to each carbonate group.

10. As a new product, a readily soluble, non-caking, non-hygroscopic alkaline detergent material in finely divided form consisting principally of a hydrated complex of trisodium phosphate and sodium carbonate, said product containing about 20% of water in stable combination and having initially a ratio of phosphate groups to carbonate groups of from about 1.2:1.

11. As a new product, a readily soluble, non-caking, non-hygroscopic alkaline detergent material in finely divided form consisting principally of a hydrated complex of trisodium phosphate and sodium carbonate, said product containing from about 18 to about 26% of water in stable combination and a ratio of phosphate groups to carbonate groups of from 1 to 1.25:1.

12. As a new product, a readily soluble, non-caking, non-hygroscopic alkaline detergent material in finely divided form consisting principally of a hydrated complex of trisodium phosphate and sodium carbonate, said product containing from about 18 to about 26% of water in stable combination and a ratio of 0.5 to 1.25 phosphate groups to each carbonate group.

13. As a new product, a readily soluble, non-caking, non-hygroscopic alkaline detergent material in finely divided form consisting principally of a hydrated complex of trisodium phosphate and sodium carbonate, said product containing from about 20 to about 23% of water in stable combination and a ratio of from 1 to 1.25 phosphate groups to each carbonate group.

14. The method of forming a stable alkaline detergent compound comprising principally a hydrated sodium phosphate and carbonate complex which comprises admixing a trisodium phosphate and a sodium carbonate compound of the class consisting of sodium carbonate and sodium sesquicarbonate and their hydrates in proportions to provide a ratio of from about 0.5 to about 1.8 phosphate groups to each carbonate group, adding water to the mixture in proportions of from about 45 to about 150% by weight of the mixture to at least form a slurry and dehydrating the resulting mixture to form a normally solid, pulverizable product containing in stable combination from about 20 to about 23% of water.

LLOYD A. HALL.  
CARROLL L. GRIFFITH.

CERTIFICATE OF CORRECTION.

Patent No. 2,142,870.

January 3, 1939.

LLOYD A. HALL, ET AL.

It is hereby certified that error appears in the printed specification of the above numbered patent requiring correction as follows: Page 3, first column, line 51, for "10<sup>10</sup> cm." read 10<sup>-10</sup> cm.; and that the said Letters Patent should be read with this correction therein that the same may conform to the record of the case in the Patent Office.

Signed and sealed this 28th day of February, A.D. 1939.

(Seal)

Henry Van Arsdale.  
Acting Commissioner of Patents.